

Jan. 10, 1956

N. F. MEIER  
METHOD FOR BREAKING-UP AN ANNULAR  
CORE OF FERROMAGNETIC MATERIAL  
Filed Sept. 8, 1952

2,730,471



INVENTOR  
NICOLAAS FREDERIK MEIER

BY

*Fred M Vogel*

AGENT

# United States Patent Office

2,730,471

Patented Jan. 10, 1956

1

2,730,471

## METHOD FOR BREAKING-UP AN ANNULAR CORE OF FERROMAGNETIC MATERIAL

Nicolaas Frederik Meier, Eindhoven, Netherlands, assignor to Hartford National Bank and Trust Company, Hartford, Conn., as trustee

Application September 8, 1952, Serial No. 308,488

Claims priority, application Netherlands October 1, 1951

3 Claims. (Cl. 148—9)

Known methods for producing closed ferromagnetic cores include placing a winding on disassembled core segments and then assembling the segments into a closed core. The pieces of the core should preferably fit together with a minimum airgap. For this purpose it has been proposed to break a core, produced by moulding powdered iron, by applying a suitable mechanical force thereto.

The invention relates to a method for breaking a circular core made of a ferromagnetic polyoxide of spinel structure of iron and other metals. This material is usually obtained by sintering and is comparatively hard and brittle. When a circular core of this material is broken mechanically the break surfaces are irregular and the core often breaks in a great many pieces. According to the invention these disadvantages are obviated in that the core is split-up by local thermal action.

Preferably the core is locally heated by a plurality of small oxy-hydrogen flames which are located along a given line, until the material cracks as a result of the unequal heating.

In order that the invention may be clearly understood and readily carried into effect, it will now be described in detail with reference to the accompanying drawing in which the process according to the invention is illustrated.

An annular core 1 produced by sintering a mixture of iron oxide and other metal oxides of cubic structure lies on a disc or table 3 which is preferably rotary. Arranged near the edge of the disc 3 is an oxyhydrogen burner 5, which yields a plurality of small flames (7) situated along a vertical line. These flames are directed to the line on the circumference of the ring 1, at which splitting-up is wanted, and which may have been marked beforehand by a chalkline. The ring cracks along this line after a few seconds as a result of the unequal heating in which the outside of the ring is heated to a much higher degree than the inside.

The break surface is comparatively smooth and only

2

in exceptional cases do small fragments of the material fly off, so that even in rapid production, the reject percentage is limited to a very low value. With the ring occupying a position in which it has turned on its axis through approximately 180°, the process is repeated, after which the ring can be dismantled in two pieces, which after the windings have been placed in position, the ring can be exactly reassembled.

The method described above is particularly suited for mass production because the rings that are to be broken, need only be placed on the table 3 at approximately the correct point and in about the required position and moved by rotation of the table 3 through a given angle so as to be arranged in front of the burner 5, whereupon splitting takes place spontaneously within a few seconds.

Heating may be effected by means of the gas flame. As an alternative it may be effected by means of an electrically heated incandescent wire or the entire ring may be heated and locally chilled by contact with a strongly cooled body.

As a further alternative the circular core may be caused to crack at one point by thermal action and by forcing apart the two ends thus obtained to produce another fracture of the ring at a point spaced about 180° from the first fracture. If necessary the ring may be scored prior to breaking the ring the second time.

What I claim is:

1. A method of breaking an annular core made of ferromagnetic polyoxide of spinel structure of iron comprising placing a heat source adjacent said core and locally heating said core to thereby split the same along at least one predetermined line.

2. A method of breaking an annular core made of ferromagnetic polyoxide of spinel structure comprising placing a heat source adjacent said core and locally heating said core by means of a plurality of small flames arranged in a line.

3. A method of breaking an annular core made of ferromagnetic polyoxide of spinel structure comprising locally heating said core by means of an incandescent wire arranged adjacent a predetermined line on said core.

## References Cited in the file of this patent

### UNITED STATES PATENTS

|           |          |               |
|-----------|----------|---------------|
| 566,436   | Woodruff | Aug. 25, 1896 |
| 684,686   | Grotz    | Oct. 15, 1901 |
| 1,025,029 | Sutton   | Apr. 30, 1912 |
| 1,194,124 | Barrow   | Aug. 8, 1916  |
| 1,251,541 | Knight   | Jan. 1, 1918  |
| 1,494,003 | Malcher  | May 13, 1924  |
| 1,887,974 | Barrow   | Nov. 15, 1932 |
| 2,283,251 | Gunther  | May 19, 1942  |